

July 30, 1929.

C. A. HALLAM

1,722,372

METHOD OF RECLAIMING METAL PORTIONS OF ELECTRICAL APPARATUS

Filed March 26, 1926



Patented July 30, 1929.

1,722,372

# UNITED STATES PATENT OFFICE.

CECIL ALFRED HALLAM, OF LA GRANGE, ILLINOIS, ASSIGNOR TO WESTERN ELECTRIC COMPANY, INCORPORATED, OF NEW YORK, N. Y., A CORPORATION OF NEW YORK.

## METHOD OF RECLAIMING METAL PORTIONS OF ELECTRICAL APPARATUS.

Application filed March 26, 1926. Serial No. 97,638.

This invention relates to methods of reclaiming metal portions of electrical apparatus, and more particularly to methods of reclaiming the metal portions of electrical condensers, such as are used in telephone systems.

In some types of electrical condensers used in telephone systems, alternate thin sheets of metal foil or other electrical conducting material and waxed paper or other forms of dielectric are tightly wound into a compact form around a pair of electrical terminals and sealed in a metal container. When such condensers become damaged or outlive their usefulness they are replaced by new condensers, but it has heretofore been impractical to satisfactorily reclaim in a commercial way the metal portions of the impaired condensers.

The objects of the present invention are to provide a simple, economical and efficient method of reclaiming the metal portions of electrical apparatus.

According to the main features of the invention, a number of condensers are placed in a foraminous drum and the sealing compound, which holds the units in the containers, is ignited to furnish the sole source of heat for melting the metal foil and the solder joining portions of the containers. When the compound ceases to burn, the drum is rotated to separate the units from the containers, the melted metal being collected in a suitable receptacle and the charred paper serving to prevent oxidation of the molten metal during the burning of the sealing compound and during the collection of the molten metal. After the molten metallic portion is collected, the unmelted containers and terminals are removed from the drum and baled.

The invention will be more fully understood from the accompanying drawings, in which—

Fig. 1 is a front elevation of a mechanism embodying the invention and which may be used for performing the process, part of the mechanism being broken away to illustrate the structure of the drum;

Fig. 2 is a side elevation thereof, and

Fig. 3 is an enlarged, diagrammatic, longitudinal section of a typical electrical condenser of the type used in telephone systems.

In the drawings in which like numerals designate similar members throughout the several views, the numeral 10 refers generally to a refractory housing preferably made of

fire brick suitably reinforced by metal girders. The housing consists of sides 11, back 12, top 13, and inclined bottom 14. The front of the housing is provided with a downwardly extending portion 15 and an upwardly extending portion 16 leaving a large charging aperture 18. The charging aperture 18 is normally covered by a vertically sliding door 17 to which is attached a wire cable 19. This cable passes over a pair of pulleys 20 and is also attached to a counter-balance 21. This counter-balance 21 is of substantially the same weight as the door 17 so that the door may be readily raised. The door is guided in its vertical path by a pair of U-shaped channel bars 70 22 and is provided with a suitable handle 23. A tapping pipe 24 extends through the front portion 16 of the housing near the inclined bottom 14. It is to be noted that the bottom 14 is inclined toward the tapping pipe 24, 75 from the back toward the front, and also from the right toward the left, as seen in Fig. 1, so that all of the molten metal which collects on the bottom 14 may be withdrawn. A stack 25 extends from the top 13 upwardly 80 to a suitable height and the stack is provided with a damper 26 for regulating the draft. A gas burner 27 extends through the left hand wall 11 of the housing, as seen in Fig. 1, which burner is connected to a gas main. 85

A hollow water-cooled shaft 28 extends from side to side through the housing and is supported by a pair of standards 29 fitted with anti-friction bearings 30 of any suitable type. A pulley 31 is keyed to the shaft 28 and the shaft is rotated by means of a belt 32 passing over the pulley 31 and connected to a suitable source of power. Mounted on the shaft 28 within the housing 10 is a foraminous drum 33, the periphery of which is provided with a plurality of holes 35. The drum 33 is fitted with a charging door 36 which is fastened to the drum by means of lugs 37 fitting over bolts 38.

The condensers to be reclaimed are indicated in Fig. 1 by the numeral 45. These condensers, which are shown in detail in Fig. 3, consist of a metallic container 40 made of tinned metal soldered together, within which casing are a pair of conductors 41 about which are tightly wound alternate layers of very thin metal foil 43, such as tin foil and waxed or paraffined paper 42. The resulting roll is sealed in the container by a suitable binder 44 made of asphalt and resin. 110

It is thought that a description of the apparatus and its operation will show in detail the manner in which the new process is practiced. In the operation of the apparatus, 5 the door 17 is raised to expose the foraminous drum 33. The drum is rotated until the charging door 36 is in the position shown in Fig. 2, the door 36 is then removed and the condensers to be reclaimed placed in the 10 drum. The door 36 is then replaced, the door 17 closed, and the gas burner 27 lighted to start the melting and burning of the binder. When the binder is ignited the gas burner is 15 extinguished. The binder and a part of the waxed paper continue to burn and thereby furnish all of the heat necessary to melt the solder from the containers and the metal foil of the condenser proper, the containers and terminals remaining unchanged. As soon as 20 the binder ceases to burn, the drum is rotated causing the containers to fall apart and to remove the condenser units therefrom. During the rotation of the drum, the resulting charred paper and the molten metal fall 25 through the perforations in the drum, into the lower portion of the furnace, and onto the inclined bottom 14. The molten metal is withdrawn through the tapping pipe 24 into a suitable mold. After all of the molten 30 metal and paper have been removed, the rotation of the drum is stopped and the containers and terminals are removed therefrom. The containers and terminals are allowed to cool and then compressed in bales.

Only a part of the paper in the condensers burns, the remainder being merely charred, thereby producing a suitable non-oxidizing material substantially enclosing the globules of molten metal produced from the foil during 35 the burning operation. The particles of carbon produced from the paper fall into the lower portion of the furnace with the molten metal and also serve to prevent oxidation of the molten metal collected therein. It is believed 40 that the presence of charred paper is one of the principal factors in making the method a success, while, of course, the fact that no heat is necessary except that generated by the burning of the binder and a portion 45 of the waxed paper, makes the process very economical.

What is claimed is:

1. A method of reclaiming metallic material enveloped by combustible substances 50 which consists in igniting one of said combustible substances to render said metallic material fluid and to reduce the other combustible substance to prevent oxidation of the metallic material, agitating the mixture

to cause the separation of the metallic material, and depositing the residue of the combustible substance and the metallic material in the same receptacle. 60

2. A method of reclaiming metallic material enveloped by combustible materials, 65 which consists in burning one of the combustible materials to furnish heat to melt the metallic material, converting the other combustible material into a reducing medium for the metal, and agitating and sifting the 70 remaining material to separate the molten metal and the reducing medium from the residue. 75

3. A method of reclaiming metal portions from composite articles, comprising metal portions and non-metallic combustible material, which consists in igniting the combustible material of the articles to heat the articles, subjecting the articles to a reducing atmosphere, and agitating the heated articles 80 to separate the remaining portions. 85

4. A method of reclaiming metal portions from composite articles, comprising metal portions and non-metallic combustible material, which consists in igniting the combustible material of the articles to heat the articles, limiting the amount of oxygen present to effect incomplete combustion, and agitating the heated articles to separate the remaining portions thereof. 90

5. A method of reclaiming separately metal portions of articles, comprising a metal container enclosing metal of a lower melting point wrapped in a combustible material, initially igniting the combustible material to heat the assembled articles and thereby melt the metal of the lower melting point, limiting the amount of oxygen present to effect incomplete combustion, agitating the heated articles to disintegrate the containers 95 from the residue, and separately collecting the containers and the molten metal and residue of the combustible material. 100

6. A method of reclaiming metal portions from composite articles, comprising metal portions and non-metallic combustible material, which consists in placing said articles in a container, igniting the combustible material of the articles while the container is stationary to heat the articles, limiting the 110 amount of oxygen present to effect incomplete combustion, and agitating the container after combustion ceases to separate the remaining portions thereof. 105

In witness whereof, I hereunto subscribe my name this 12th day of March A. D., 1926. 115

CECIL ALFRED HALLAM.